

E. M. CAFFALL.  
PROTECTION OF STEEL.  
APPLICATION FILED OCT. 16, 1910.

1,098,368.

Patented June 2, 1914.



WITNESSES

*J. E. Caffall  
E. Bradford*

INVENTOR

Edward M. Caffall.

BY

*ATTORNEY*

# UNITED STATES PATENT OFFICE.

EDWARD MAY CAFFALL, OF SPARKILL, NEW YORK.

## PROTECTION OF STEEL.

1,098,368.

Specification of Letters Patent.

Patented June 2, 1914.

Application filed October 15, 1910. Serial No. 587,184.

To all whom it may concern:

Be it known that I, EDWARD M. CAFFALL, a citizen of the United States, and resident of Sparkill, in the county of Rockland and 5 State of New York, have invented certain new and useful Improvements in the Protection of Steel, of which the following is a specification.

My invention relates to a process for protecting steel products, particularly such as beams and rails, from corrosion or oxidation and to apparatus for carrying out the process.

Steel as the term is commonly employed 15 denotes iron alloyed with other substances including carbon. The carbon content varies with the different grades and qualities of steel depending upon the method and materials of manufacture. Steel when exposed rapidly deteriorates by reason of corrosion sometimes local and sometimes very extensive. Various methods of preventing this such as by paint and plating with other non-oxidizable metals are in vogue. The 20 corrosion is variously attributed to chemical and to electrical action. While plating processes are satisfactory to a certain degree they are very expensive. Ordinary paint while effective to a certain extent is itself 25 subject to oxidation and readily flakes off and this leaves the surface of the metal exposed to local action.

It is my object to provide a method for 30 coating steel which is inexpensive and which will result in a permanent and practically indestructible product.

My improved method contemplates immersing the steel while hot in a bath of paraffin then withdrawing the steel and allowing it to cool. The temperature of the bath should be about 150° F. or somewhat higher and the temperature of the steel considerably higher but below 600° F. If the temperature is much higher than this the 45 bath is likely to be ignited. The steel to be treated should be practically free from scale and for this reason I prefer to treat members such as beams immediately after they leave the final finishing rolls of the mill 50 and before scale forms. As they come from these rolls if the temperature is above 600° F. they should be allowed to cool slightly. As they are plunged into the bath the temperature of the steel falls and the metal contracts. In this way the hot paraffin is 55 drawn into the pores of the steel to a con-

siderable extent and becomes so anchored that there is no tendency for it to peel off. The paraffin coat formed by this process is more or less flexible so that the bending of 60 the steel does not crack it off. The temperature of the bath should be maintained substantially constant by suitable means. Preferably when the beams are withdrawn from the bath they are allowed to drain adjacent thereto so that any excess of paraffin 65 adhering to the beams will run back into the bath.

The drawing is a diagrammatic illustration of apparatus for carrying the invention into effect in treating beams and similar products.

The reference numeral 1 indicates the final pair of finishing rolls of a mill. These are driven by any suitable source of power 70 as for instance from the countershaft 2. The beams after passing through the rolls are laid upon the floor 3 or any other suitable support. A suitable form of conveyer is preferably provided for taking up the 75 beams as they come from the finishing rolls, taking them to the bath, immersing them therein and withdrawing them therefrom. In the form shown this consists of a suitable pair of tongs or other device such as 4 operated from the traveling hoist 5 which runs 80 on a rail 6. The bath is contained in a tank 7 of any suitable construction for instance of metal arranged in a convenient location adjacent to the finishing rolls. This tank is 85 heated in any suitable manner for instance by means of movable fire boxes 8, 8 so that the fires may be withdrawn if the temperature of the bath gets too high and may be reapplied when the temperature gets too 90 low. In this connection it will be noted that as the steel beams or other members are of a considerably higher temperature than the bath they will have a tendency, while the process continues, to impart sufficient heat 95 to the bath to maintain it above the minimum temperature without the use of the fires 8, 8. If however, the quantity of material being treated is small or the process operated intermittently, it will be necessary 100 to apply heat to the bath in order to maintain the desired minimum temperature. The paraffin will penetrate any slight scale which may form between the time the steel leaves the rolls and enters the bath. The 105 members are left in the bath if necessary, a short time say—from one to five seconds and

are then withdrawn and laid upon a suitable rack or support such as the inclined trough 9 from which the excess of paraffin may run back into the tank so as to avoid 5 wasting of the paraffin and unnecessary depletion of the bath.

I have found that the process operates more successfully and that the product is superior when a certain per cent. of some 10 carbonaceous material such as lampblack is mixed with the paraffin in the bath. The proportion of lampblack employed may vary from say—2 ounces to the gallon of paraffin up to say—a pound of lampblack to a gallon 15 of paraffin depending upon the results desired. The lampblack gives body to the coating and durability so that it is able to withstand a greater amount of wear and tear without materially injuring the coating 20 or exposing the surface of the metal. A percentage of diatomite may also be employed either with the lampblack or supplementary thereto and in about the same proportions. Diatomite is practically a non- 25 conductor of heat and will enable the product to withstand a great amount of abrasion. The diatomite may be applied in the bath, with the lampblack or in a separate bath, either as a substitute for the whole or a part 30 of the lampblack in some cases or supplementary thereto in other cases. I have also found that when steel beams or other members have been treated with paraffin and lampblack as herein described an especially 35 effective result is obtained by dusting the coated steel with diatomite while the steel is hot and the paraffin is still soft. As the steel and paraffin cools the diatomite becomes strongly embedded in the paraffin.

40 When beams or steel members are used in building constructions it is often necessary to unite two or more parts by means of rivets. In practising my process paraffin is

applied to each end of each rivet as the rivet is being finally upset and while hot 45 and by this means every part of the metal surface is coated and such spaces as exist between the rivets and the beams are filled with the wax.

The paraffin is practically unaffected by 50 acids or the weather and not subject to oxidation and when applied as herein set forth prevents any corrosion or oxidation of the steel. Even when the surface of paraffin is worn off there is a sufficient quantity of the 55 paraffin left in the pores of the steel to prevent any corrosion other than the most minute and superficial.

Steel, coated according to my invention may be painted if desired and ordinary 60 paint will adhere thereto.

What I claim is:—

The process of protecting steel from corrosion by means of paraffin which consists in immersing uncoated steel in an open bath 65 of melted paraffin the temperature of the steel being considerably above the melting point of the paraffin and below the ignition point of the paraffin, maintaining the temperature of the paraffin substantially constant, leaving the steel in the bath for a sufficient length of time to permit the steel 70 to be cooled somewhat and absorb the paraffin into the steel, and withdrawing the steel from the bath while the steel is still at 75 a temperature above the melting point of the paraffin and allowing the steel to drain and cool outside the bath.

Signed at New York, in the county of New York and State of New York this 13th 80 day of October A. D. 1910.

EDWARD MAY CAFFALL.

Witnesses:

CORNELIUS W. WICKERSHAM,  
ROBT. S. ALLYN.